

# UNITED STATES PATENT OFFICE.

GUSTAV LANGENHAGEN, OF LEIPSIC, SAXONY, GERMANY.

## LEATHER-POLISH.

SPECIFICATION forming part of Letters Patent No. 406,102, dated July 2, 1889.

Application filed January 26, 1887. Serial No. 225,570. (No specimens.)

*To all whom it may concern:*

Be it known that I, GUSTAV LANGENHAGEN, of Leipsic, in the Kingdom of Saxony and German Empire, have invented a new and useful Improved Leather-Polish, of which the following is a specification, no patents having been obtained by me anywhere for this invention.

My invention relates to improved leather-polish.

All leather-polishes in use until now show many deficiencies. Pure coal-tar oils—as vaseline, for instance—are susceptible of very little absorption, and thereby render the leather dry and flabby. Mixtures of coal-tar oils—as, for instance, mixture of heavy coal-tar oil and wax—show the same deficiency, while pure animal and vegetable fats are liable to get rancid, and therefore are very noxious. Heretofore the exact proportion to prevent rancidity and insure a uniform absorption has never been attained by mixing them. The mixture hereinafter detailed is the result of exact trials, and cannot be varied without causing considerable prejudice to its quality. As most important for securing the absorption of the mixture and the conserving the

gloss of the leather, and nevertheless unknown until now, there is especially to be mentioned a considerable addition of oil of turpentine. 30 The coloring substances are dissolved.

The leather-polish consists of the following components: Forty per cent. of carnauba-wax, one per cent. of steatite, thirty per cent. of oil of turpentine, five per cent. of aniline, 35 (nigrosine,) two per cent. of Congo black, eight per cent. of almond-kernel oil, four per cent. of beeswax, and ten per cent. of ozocerite.

What I claim, and desire to secure by Letters Patent of the United States, is— 40

A leather-polish consisting of forty per cent. of carnauba-wax, one per cent. of steatite, thirty per cent. of oil of turpentine, five per cent. of aniline, (nigrosine,) two percent. of Congo black, eight per cent. of almond-kernel oil, four per cent. of beeswax, and ten per cent. of ozocerite, substantially as described. 45

In witness whereof I have hereunto set my hand in presence of two witnesses.

GUSTAV LANGENHAGEN.

Witnesses:

CARL SËYFFERT,  
CARL BORNGRAEBER.